

Patented June 2, 1931

1,808,184

## UNITED STATES PATENT OFFICE

DEAL H. TOMPKINS, OF NITRO, WEST VIRGINIA, ASSIGNOR TO THE RUBBER SERVICE LABORATORIES COMPANY, OF AKRON, OHIO, A CORPORATION OF OHIO

## CLEANING AND PRESERVING OF METALLIC SURFACES

No Drawing.

Application filed June 30, 1930. Serial No. 465,070.

The present invention relates to the cleaning and preservation of metallic surfaces, wherein the metal is in contact with a liquid of an acid nature. More particularly, the 5 invention relates to the prevention of excessive pitting and embrittlement of a metal when subjected to a pickling process.

Certain objects of the invention are to prevent the acid pickle liquor from attacking 10 clean portions of the surface of a metal; to obviate over-pickling, embrittlement and pitting of the articles treated; to minimize the amount of metal lost in pickling; to increase the efficiency of the pickling operation and to 15 prolong the effective life of the pickling bath and particularly to speed the pickling operation. Other and further objects of the invention will be apparent from the following description and accompanying examples.

20 In the art of pickling, the metal is treated with a dilute acid to remove oxides such as rust, scale, and other deposits, after which the metal is preferably washed with water and dipped into an alkaline bath to remove 25 the last traces of free acid. The acid removes the rust and scale, but unfortunately, from the pickling standpoint, it attacks the cleaned metal itself thereby causing loss of metal and producing an evolution of hydrogen gas, 30 which escapes into the air, carrying with it a fine spray of the pickling bath and producing an atmosphere possessing corrosive properties and one which is highly injurious to health.

35 By the present invention, these objectionable features of the pickling process are substantially overcome or reduced to a minimum. To accomplish the objects set forth in accordance with the present invention, there is 40 added to the pickling bath a regulating agent or ingredient which acts to restrain the action of the acid from attacking clean metal but assists in removing the rust, scale and other deposits, or in other words it selectively 45 removes such materials without appreciably attacking the clean portions of the metal.

The pickle regulator or inhibitor, as disclosed in the present application, comprises a sulfuric acid derivative of a reaction product 50 of sulfur dioxide and an aldehyde-amine re-

action product and preferably a sulfuric acid derivative of a reaction product of sulfur dioxide and an aldehyde derivative of a Schiff's base; that is, a product formed by reacting an aldehyde with a Schiff's base, adding sulfur dioxide thereto and treating the product so formed with sulfuric acid of any concentration necessary to produce sulfonation at the reaction temperature employed. 55

In the examples hereinafter set forth for carrying out the metal pickling process, conditions were imposed which duplicated, so far as possible, those commonly followed in commercial practice, so far as concerned acid concentrations and temperatures employed. 60

65 Test pieces of steel approximately 4' x 3', 30 gauge hot rolled tin plate stock were then immersed in approximately 500 c. c. of a water solution of sulfuric acid containing approximately 8% by weight of 66° Bé. acid to which had been added a small quantity of one of the preferred type of inhibitors. The loss in weight of the steel test pieces resulting from maintaining the strips in the pickle bath in the manner described for a definite period of time was then determined. The temperature of the pickling bath was maintained at from 176 to 185° F. (80 to 70 85° C.). For the acid concentration set forth, commercial practice is to pickle at approximately 150 to 190° F. (66 to 88° C.). The results so obtained were compared with similar tests wherein the steel pieces were subjected, under the conditions set forth, to the action of an acid solution of the strength and for the time specified above, but containing no inhibitor. 75

80 One method whereby one of the preferred class of compounds, for example a sulfuric acid derivative of the reaction product of sulfur dioxide and an aldehyde derivative of a Schiff's base, was prepared as follows:

85 Substantially one molecular proportion of the product formed from the reaction of substantially three molecular proportions of acetaldehyde and substantially two molecular proportions of aniline, according to the method set forth in U. S. Patent No. 1,659,152 90 granted to Clayton Olin North, was dis- 95

100

solved in an organic solvent, for example, a quantity of acetone equal to one-third of the weight of the aldehyde-amine product. Substantially one-half a molecular proportion of sulfur dioxide was passed thereinto at a rate slow enough for complete absorption and combination to take place while agitating and maintaining a temperature of approximately 30 to 60° C. To the product thus formed, substantially one molecular proportion of sulfuric acid, preferably having an acid strength of 75% was added at a temperature of substantially 50 to 70° C. After the addition of the sulfuric acid was completed, the water present and the solvent employed, for example acetone, were removed preferably by evaporation. The product prepared in the manner described, after cooling was a brittle resin, which formed a fine powder when ground that was readily soluble in a pickle liquor as for example dilute sulfuric acid. A sample of the material prepared as described above was incorporated in a pickling bath in the manner hereinbefore described. Thus a steel test piece 3" x 4", 30 gauge hot rolled tin plate stock, exposing 24 square inches of surface and weighing 17.5228 grams, was found to lose but 0.0173 grams after 20 minutes pickling in an 8% sulfuric acid solution containing 0.12 grams of the inhibiting product just described. A similar test piece weighing 17.0100 grams and treated in the same manner, but without the use of any inhibitor lost 0.2997 grams. Thus, when the sulfuric acid derivative of the reaction product of sulfur dioxide and the product formed by reacting substantially three molecular proportions of acetaldehyde and substantially two molecular proportions of aniline is employed as an inhibitor, the loss in weight per square inch of surface exposed corresponds to 0.00072 grams whereas when no inhibitor is used the loss per square inch of surface exposed corresponds to 0.0125 grams. A greater saving in metal losses results from the use of a larger amount of the inhibitor. Moreover, the steel plates pickled in the presence of the inhibitor set forth are clean and not stained upon removal from the bath.

Although it is desirable that the preferred inhibitor be prepared in the presence of an organic solvent, as for example acetone, benzene and the like, it is not imperative that a solvent be employed. Thus a sulfuric acid derivative of the reaction product of sulfur dioxide and the product formed by reacting substantially three molecular proportions of acetaldehyde and substantially two molecular proportion of aniline was prepared by passing substantially one-half a molecular proportion of sulfur dioxide slowly into the aldehyde-amine compound with agitation at a temperature of substantially 60 to 70° C. To the product so formed ap-

proximately one molecular proportion of sulfuric acid having an acidity of approximately 75% was added with agitation at a temperature of approximately 90 to 100° C. A sample of the above identified material was incorporated in a sulfuric acid pickling bath in the manner previously described. The following table shows a comparison between the loss in weight of the test strips, after immersion in the pickling bath for twenty minutes, when the inhibitor just described was employed and when no inhibitor was employed.

Table I

3" x 4", 30 gauge hot rolled tin plate stock pickled twenty minutes in 8% sulfuric acid at 80° C.

| Amount of inhibitor employed | Weight of metal strip before pickling | Weight of metal strip after pickling | Weight loss in grams per sq. in. of surface exposed |
|------------------------------|---------------------------------------|--------------------------------------|-----------------------------------------------------|
| Gram                         | Grams                                 | Grams                                | Grams                                               |
| 0.12                         | 15.4302                               | 15.4200                              | 0.000495                                            |
| 0.12                         | 17.4634                               | 17.4544                              | 0.000375                                            |
| 0.12                         | 17.2150                               | 17.2065                              | 0.000354                                            |
| 0.12                         | 16.8387                               | 16.8288                              | 0.000412                                            |
| None.                        | 16.8081                               | 16.5000                              | 0.012887                                            |
| None.                        | 16.1870                               | 15.8955                              | 0.012145                                            |

Average loss with inhibitor 0.000391 grams per sq. in.

Average loss without inhibitor 0.012491 grams per sq. in.

From the results set forth in Table I it is apparent that the average loss in weight when no inhibitor is employed is approximately thirty-four times greater than the average loss resulting when the inhibitor set forth is employed in the pickle bath described.

Other sulfuric acid derivatives of the reaction products of sulfur dioxide and aldehyde-amine products, and preferably sulfuric acid derivatives of the reaction products of sulfur dioxide and aldehyde derivatives of Schiff's bases have been prepared in a manner analogous to that hereinbefore set forth and tested as inhibitors in a pickling bath in the manner described.

Thus, the sulfuric acid derivatives of the sulfur dioxide reaction products of a Schiff's base and of aldehyde derivatives thereof as set forth hereinafter were prepared and the final product so obtained employed in a pickling bath and tested in the manner described. The products referred to in the results set forth in Table II, as inhibitors A to G inclusive, represent the sulfuric acid derivatives of the sulfur dioxide reaction product of the following bases:

*Compound A.*—Substantially three molecular proportions of acetaldehyde and two molecular proportions of ortho-toluidine.

*Compound B.*—Anhydro formaldehyde aniline.

*Compound C.*—Substantially three molecular proportions of butylaldehyde and one molecular proportion of aniline.

5 *Compound D.*—Substantially one molecular proportion of 2-4 diamido diphenylamine and three molecular proportions of heptaldehyde.

10 *Compound E.*—Substantially three molecular proportions of heptaldehyde and one molecular proportion of aniline.

*Compound F.*—Substantially one molecular proportion of formaldehyde and one 15 molecular proportion of beta-naphthylamine.

*Compound G.*—Substantially three molecular proportions of butylaldehyde and one molecular proportion of ortho-toluidine.

Table II

20 3" x 4", 30 gauge hot rolled tin plate stock pickled twenty minutes in 8% sulfuric acid at 80° C.

| Inhibiting compound employed | Weight of inhibitor employed | Weight of steel strip before pickling | Weight of steel strip after pickling | Weight loss in grams per sq. inch of surface exposed |
|------------------------------|------------------------------|---------------------------------------|--------------------------------------|------------------------------------------------------|
| 25 Compound A                | Grams                        | Grams                                 | Grams                                | Grams                                                |
| Compound B                   | 0.12                         | 16.672                                | 16.655                               | 0.00071                                              |
| Compound C                   | 0.12                         | 16.810                                | 16.798                               | 0.00050                                              |
| Compound D                   | 0.12                         | 17.342                                | 17.336                               | 0.00025                                              |
| Compound E                   | 0.12                         | 17.122                                | 17.101                               | 0.00087                                              |
| Compound F                   | 0.12                         | 16.655                                | 16.649                               | 0.00025                                              |
| Compound G                   | 0.12                         | 17.503                                | 17.496                               | 0.00029                                              |
| 35 None                      | None.                        | 16.620                                | 16.604                               | 0.00058                                              |
|                              |                              | 17.0100                               | 16.7103                              | 0.01248                                              |

It is thus apparent from the data set forth that the preferred class of materials constitute an important group of inhibitors, as in all cases where one of the preferred inhibiting compounds was incorporated in the pickle liquor, there resulted a metal saving of from 96 to over 98% of the loss in weight of the steel test strips that resulted when no inhibitor was employed.

45 The preferred class of inhibiting compounds has also been employed in other pickling baths than sulfuric acid wherein materials other than iron and steel were pickled. The following example illustrates one method of pickling a nickel chromium alloy, wherein one of the preferred inhibitors, for example, the product formed by treating the reaction product of sulfur dioxide and the 55 aldehyde-amine product prepared from substantially three molecular proportions of acetaldehyde and substantially two molecular proportions of aniline with sulfuric acid in the manner previously described, was employed as an inhibitor in a hydrochloric acid pickling bath.

A piece of nickel chromium alloy wire having a composition of 80% nickel and 20% chromium, 36 inches in length, 0.036 inches 60 in diameter, having a total surface of 4.07

square inches and weighing 5.2640 grams, was coiled in the form of a spiral and immersed in approximately 500 grams of 17% hydrochloric acid containing 0.24 grams of the product formed by treating the reaction product of substantially three molecular proportions of acetaldehyde and substantially two molecular proportions of aniline with sulfur dioxide and further reacting said product with sulfuric acid in the manner hereinbefore described. After allowing the wire to remain in the pickle liquor for 20 minutes at 176° F., the loss in weight was found to be only 0.0405 grams. A test identical with that described above with the exception that the nickel-chromium wire weighed 5.3225 grams and no inhibitor was employed, showed a loss of 0.2060 grams. In other words the weight loss due to solvent action of the hydrochloric acid on the metal was only 75 one-fifth as great when the preferred inhibitor was employed as was the loss with no inhibitor present. A greater saving in metal would be realized by employing a greater proportion of the inhibitor.

80 It has further been found that other ratios of sulfuric acid, sulfur dioxide and aldehyde-amine than those hereinbefore set forth may be reacted and employed as inhibitors. Thus substantially one molecular proportion of the aldehyde derivative of a Schiff's base formed by reacting substantially three molecular proportions of acetaldehyde with substantially two molecular proportions of aniline has been reacted with varying amounts 85 of sulfur dioxide preferably in the ratios between substantially one-fifth to one molecular proportion and the material so prepared further reacted with varying concentrations of sulfuric acid preferably in ratios 90 varying between three-fourths to one and one-half molecular proportions. In all cases the materials so obtained, on incorporating 95 in a pickle bath and testing in the manner hereinbefore set forth, were found to be very desirable inhibitors.

100 Other solvents than acetone have also been employed in the preparation of the preferred class of inhibitors. For example the sulfuric acid derivative of the reaction product 105 of sulfur dioxide with the material formed from substantially three molecular proportions of acetaldehyde and substantially two molecular proportions of aniline has been prepared in a benzene medium and the resulting material on testing found to be a very desirable inhibitor.

110 Other modes of employing inhibitors of the type set forth herein in the acid pickling of metals are apparent to those skilled in the art to which this invention pertains. The products described additionally may be employed in the pickling process in the presence of foaming agents, ionizable substances or other materials ordinarily used.

What is claimed is:

1. A process of pickling iron and steel products which comprises subjecting the metal to be pickled to the action of a sulfuric acid solution containing a small proportion of a sulfuric acid derivative of a reaction product of sulfur dioxide and an aldehyde-amine product. 70
2. A process of pickling iron and steel products which comprises subjecting the metal to be pickled to the action of a sulfuric acid solution containing a small proportion of a sulfuric acid derivative of a reaction product of sulfur dioxide and an aldehyde-aromatic-amine reaction product. 75
3. A process of pickling iron and steel products which comprises subjecting the metal to be pickled to the action of a sulfuric acid solution containing a small proportion of a sulfuric acid derivative of a reaction product of sulfur dioxide and an aldehyde derivative of a Schiff's base. 80
4. A process of pickling iron and steel products which comprises subjecting the metal to be pickled to the action of a sulfuric acid solution containing a small proportion of a sulfuric acid derivative of a reaction product of sulfur dioxide and an aliphatic aldehyde derivative of a Schiff's base. 85
5. A process of pickling iron and steel products which comprises subjecting the metal to be pickled to the action of a sulfuric acid solution containing a small proportion of a sulfuric acid derivative of a reaction product of sulfur dioxide and a material formed by reacting an aliphatic aldehyde containing less than eight carbon atoms with a primary aromatic amine. 90
6. A process of pickling iron and steel products which comprises subjecting the metal to be pickled to the action of a sulfuric acid solution containing a small proportion of a sulfuric acid derivative of a reaction product of sulfur dioxide and a material formed by reacting substantially three molecular proportions of acetaldehyde with substantially two molecular proportions of aniline. 95
7. A process of pickling iron and steel products which comprises subjecting the metal to be pickled to the action of a sulfuric acid solution containing a small proportion of a product formed by reacting substantially one-half a molecular proportion of sulfur dioxide with substantially one molecular proportion of the reaction product of substantially three molecular proportions of acetaldehyde and substantially two molecular proportions of aniline and further reacting the product thus formed with substantially one molecular proportion of sulfuric acid. 100
8. A process of pickling iron and steel products which comprises subjecting the metal to be pickled to the action of a sulfuric acid solution containing a small proportion of a product formed by reacting in the presence of acetone substantially one-half a molecular propor- 105
9. A pickling bath for iron and steel products comprising a sulfuric acid solution containing a small proportion of a sulfuric acid derivative of a reaction product of sulfur dioxide and an aldehyde-amine product. 110
10. A pickling bath for iron and steel products comprising a sulfuric acid solution containing a small proportion of a sulfuric acid derivative of a reaction product of sulfur dioxide and an aliphatic aldehyde-aromatic-amine reaction product. 115
11. A pickling bath for iron and steel products comprising a sulfuric acid solution containing a small proportion of a sulfuric acid derivative of a reaction product of sulfur dioxide and an aldehyde derivative of a Schiff's base. 120
12. A pickling bath for iron and steel products comprising a sulfuric acid solution containing a small proportion of a sulfuric acid derivative of a reaction product of sulfur dioxide and an aliphatic aldehyde derivative of a Schiff's base. 125
13. A pickling bath for iron and steel products comprising a sulfuric acid solution containing a small proportion of a sulfuric acid derivative of a reaction product of sulfur dioxide and a material formed by reacting an aliphatic aldehyde containing less than eight carbon atoms with a primary amine. 130
14. A pickling bath for iron and steel products comprising a sulfuric acid solution containing a small proportion of a sulfuric acid derivative of a reaction product of sulfur dioxide and a material formed by reacting substantially three molecular proportions of acetaldehyde with substantially two molecular proportions of aniline. 135
15. A pickling bath for iron and steel products comprising a sulfuric acid solution containing a small proportion of a product formed by reacting substantially one-half a molecular proportion of sulfur dioxide with substantially one molecular proportion of the reaction product of substantially three molecular proportions of acetaldehyde and substantially two molecular proportions of aniline and further reacting the material thus formed with substantially one molecular proportion of sulfuric acid. 140
16. A pickling bath for iron and steel products comprising a sulfuric acid solution containing a small proportion of a product formed by reacting in the presence of acetone substantially one-half a molecular propor- 145

tion of sulfur dioxide with substantially one molecular proportion of the reaction product of substantially three molecular proportions of acetaldehyde and substantially two molecular proportions of aniline and further reacting the material thus formed with substantially one molecular proportion of substantially 75% sulfuric acid.

17. A process of pickling a metal which comprises subjecting the metal to be pickled to the action of a substantially non-oxidizing mineral acid solution containing a small proportion of a sulfuric acid derivative of a reaction product of sulfur dioxide and an aldehyde-amine product.

18. A process of pickling a metal which comprises subjecting the metal to be pickled to the action of a substantially non-oxidizing acid solution containing a small proportion of a sulfuric acid derivative of a reaction product of sulfur dioxide and an aldehyde-aromatic amine reaction product.

19. A pickling bath for metal products which comprises a substantially non-oxidizing mineral acid solution containing a small proportion of a sulfuric acid derivative of a reaction product of sulfur dioxide and an aldehyde-amine product.

20. A pickling bath for metal products which comprises a substantially non-oxidizing mineral acid solution containing a small proportion of a sulfuric acid derivative of a reaction product of sulfur dioxide and an aliphatic aldehyde-aromatic amine reaction product.

In testimony whereof I hereunto affix my signature.

DEAL H. TOMPKINS.

40

45

50

55

60

65